

July 30, 1935.

W. T. CRESPINEL

2,009,689

METHOD OF PRODUCING FILMS IN NATURAL COLOR

Filed Aug. 19, 1930



## UNITED STATES PATENT OFFICE

2,009,689

METHOD OF PRODUCING FILMS IN  
NATURAL COLOR

William T. Crespinel, Los Angeles, Calif., assignor, by mesne assignments, to Hughes Industries Co. Ltd., a corporation of Delaware

Application August 19, 1930, Serial No. 476,251

22 Claims. (Cl. 95—2)

My invention relates to a method of producing films in natural color, employing a positive film having two layers of sensitized emulsion superimposed on one side thereof, this film being 5 termed a "sandwich" film.

It is an object of my invention to provide a process for producing a color positive in which the image appears in natural color, and it is a further object of the invention to provide a 10 process which will give satisfactory or substantially perfect results in the production of a color film without the exercise of extreme care in the performance of the process.

It is a further object of the invention to provide a process of the above character by which a color film may be produced from color value negatives in a minimum period of time and with a relatively small expenditure of labor.

Further objects and advantages of my invention will appear throughout the disclosure of a preferred manner of performing my new process, which refers to the accompanying drawing diagrammatically showing my invention.

For the purpose of segregating the principal 25 steps of my invention, I shall in the drawing and hereinafter in the description designate same by letters.

## (A) Preparation of color value negatives

In my process I prefer to employ color value negatives representing yellow-red and blue-green values of a color image. Owing to the fact that there are many methods known to the art of color photography for the production of color 30 value negatives, and since this invention relates principally to a new process for producing a positive film in color, it is not necessary to further describe the production of the color value negatives employed in the process.

Although other types of film may be employed in the practice of my invention, I prefer to use the type of film 10 shown in the diagrammatic disclosure of step B of my invention, which consists of a transparent base, generally of celluloid, a thin primary gelatine substratum on the front face of the transparent base, a primary layer of sensitized emulsion, a secondary gelatine substratum, and an outer or secondary layer of sensitized emulsion. The primary substratum has its principal utility in securing the primary sensitized emulsion to the transparent base, and the secondary substratum serves to separate and to act as a barrier between the primary and secondary sensitized emulsion coatings. Incorporated either in the emulsions or

in the secondary substratum of the positive film 10 is a yellow dye which prevents penetration of light from one emulsion to the other.

## (B) Printing positives from color value negatives

In the printing of the positive 10, the red color value negative is placed adjacent to the transparent base, and the primary sensitized emulsion is printed by light which passes through the red color value negative, the transparent base, and the 15 primary gelatine substratum. The blue color value negative is placed adjacent to the secondary sensitized emulsion, and the secondary sensitized emulsion is printed directly from the blue color value negative. The printing of the primary and 20 secondary sensitized emulsions may be carried on simultaneously or separately.

In printing I find it advisable to differentiate between the voltage used in printing the outer and inner emulsions. To clarify this I would use 20 100 volts to the outer or secondary emulsion and 110 volts to the inner or primary emulsion. The reason for this is that it is an advantage in developing, since the developer attacks more readily the outer image and has to penetrate through to 25 the inner image, during which time the outer image is still developing, but because of the additional exposure to the inner emulsion it will develop more quickly when the developer has thoroughly saturated it.

## (C) Developing, fixing, and washing positive

This step of the process I carry on in the usual manner of developing photographic positives and have used with satisfactory results a number of 30 developers, preference among which is given to Amiddol developer, which produces so-called flat images, although good results may also be obtained from standard developers, such as Eastman developer No. 16. After treatment by the 35 developer solution, the image is fixed and then thoroughly washed, whereupon the next step of the process may be carried on with the film wet or with the film dried.

## (D) Mordanting secondary emulsion

Although it is possible to continue the operation and perform the operation of mordanting the outer or secondary emulsion while the film is still wet, I find that if the film is first dried thoroughly, 50 the coloring operations may be carried on to best advantage. The positive film is conducted through a bath or solution of potassium tri-iodide and potassium iodide characteristics with an addition of acetic acid. A suitable formula for the

mordant for basic dyes which I employ in this step of the process is as follows:

|                       |                          |
|-----------------------|--------------------------|
| Iodine resublimated   | 2 grams                  |
| 5 Potassium iodide    | 25 grams                 |
| Acetic acid (glacial) | 50 c. c. of 10% solution |
| Water to make         | 500 c. c.                |

The film is allowed to remain in this solution for a period of time sufficient to penetrate through and bleach the surface image or secondary sensitized emulsion. The secondary gelatine substratum separating the two layers of emulsion acts as a retardant to the mordanting solution and will prevent the mordanting solution from entering the silver image of the primary sensitized emulsion. If the exposure and development are carefully adjusted, I find that this operation may be consistently performed without affecting the image of the primary sensitized emulsion in a time of approximately one and one-half minutes. The film is then run into a wash tank of running water to thoroughly wash out the excess of mordanting solution. The above mordanting formula is the preferred proportion, but I have found that the proportions may be considerably varied without greatly affecting the results obtained. The potassium iodide is the predominating chemical employed, and the potassium tri-iodide and acetic acid are the ancillary chemicals. I find that the following proportions may be satisfactorily employed:

|                     |                                 |
|---------------------|---------------------------------|
| Iodine resublimated | 1 1/4 to 2 grams                |
| Potassium iodide    | 25 to 50 grams                  |
| 35 Acetic acid      | 50 to 100 c. c. of 10% solution |
| Water to make       | 500 c. c.                       |

#### (E) Arresting of mordanting action

From the wash tank of the previous step of the process the film is carried into a solution of an arresting agent of bisulphite character, such as either potassium metabisulphite or sodium bisulphite, good results being obtained where a 10% solution is employed. In this solution the action of the mordanting solution is immediately stopped, and the mordanting solution is cleared from the film. This operation requires from one-half minute to one minute, depending upon the strength of the arresting solution. The film is again thoroughly washed in a bath of running water to remove the clearing or arresting solution.

#### (F) Red-dyeing of secondary emulsion

The secondary emulsion, after treatment by the mordanting solution, is subjected to a red basic dye solution which is preferably in the form of a bath through which the film is carried. In this red-dyeing bath I employ safranine Y, Shultz & Julius index No. 679, or chrysoidine Y, Shultz & Julius index No. 33, or a solution containing proper amounts of both of them. The preferred formula for this bath is as follows. Stock solutions are first prepared as follows:

|                |                              |
|----------------|------------------------------|
| 65 Safranine Y | 1 gram in 100 c. c. of water |
| Chrysoidine Y  | 1 gram in 100 c. c. of water |

From this stock solution I prepare the red-dyeing bath in the following proportions:

|                  |          |
|------------------|----------|
| 70 Chrysoidine Y | 90 c. c. |
| Safranine Y      | 10 c. c. |
| Acetic acid      | 1 c. c.  |

Where this solution is made in accordance with the above formula, the red-coloring action may

be accomplished by running the film into the bath thereof for a period of approximately three minutes, during which time the mordant absorbs the basic dye and becomes or is converted into a brilliant orange-red.

5

#### (G) Removal of excess red-dye

The film is now carried into running water which removes the excess red-dyeing solution from the film, leaving the silver deposit forming the image of the secondary emulsion colored orange-red, the strength of the color being in proportion to the quantity of the silver deposit. If the correct dyes are used and in their correct proportions, substantially as noted above, this removal of the excess red-dye will take approximately five minutes. At this time the film carries a top image with a basic red dye and a lower image in the primary sensitized emulsion which is still black and white, the two images being separated by the intermediate substratum.

20

#### (H) Blue-toning primary emulsion

The film is now carried into a ferric solution for the purpose of coloring the image of the primary emulsion. For this purpose I employ a solution of low acid content. I find that great care must be exercised in the use of the more potent acids, such as hydrochloric acid, which affect the iodide mordant so as to increase the opacity of the red-dye image, which, if correctly executed, is very transparent. For this purpose I prefer to use a ferric bath in which acetic acid is substituted for the usual hydrochloric acid, the ferric bath being made substantially in accordance with the following formula:

|                      |                          |
|----------------------|--------------------------|
| Ammonium persulphate | 3 1/2 grams              |
| Ferric alum          | 2 1/2 grams              |
| Ferricyanide         | 2 1/2 grams              |
| Acetic acid          | 10 c. c. of 10% solution |
| Water to make        | 1000 c. c.               |

This bath will not affect the red-dye image of the secondary emulsion but will readily penetrate through the secondary substratum and in four or five minutes convert the image of the primary substratum to a blue-tone image. After being subjected to the ferric solution for a length of time gauged in accordance with the strength of the solution, the film is again washed in running water.

#### (I) Clearing or fixing the blue-tone primary emulsion

Since the red dyed image is relatively transparent and the ferric image is somewhat opaque, it is necessary to fix the ferric image to bring its transparency into a suitable balance with the red-dye image. However, the ordinary hypo fixing bath cannot be used for this purpose since it destroys the silver iodide mordant so as to result in release of the red dye from the image of the secondary emulsion. For the purpose of fixing the ferric image I employ a 10% solution of potassium iodide. Since the mordanted image of the secondary emulsion is composed of silver iodide, this fixing solution has no effect upon the red-dye image but will effectively clear the blue image of the primary emulsion in a period of about three minutes, after which the film is again washed. An added advantage of the use of this bath is the fact that if it were possible to use a hypo sulphite fixing solution, a prolonged washing would then be necessary to remove all traces of hypo from the film itself, and

75

this prolonged washing would impair both of the colored images. Thus, where the iodide clearing solution is used, a brief wash of from two to four minutes is sufficient and completes the 5 operation of producing the positive film in color.

If a sound track is to be printed on the positive film, I find it advisable to print such sound track by placing the sound negative against the secondary emulsion and to print same with greater 10 light exposure than that used in the printing of the red image, in order that the light will penetrate and also expose the sound track portion of the primary emulsion.

A transparent dyed image is not a suitable medium for sound recording because the rays from the exciter lamp, which is part of the projector equipment, will readily penetrate the dyed image, and the resulting sound would be very weak and poor in quality. The sound track could be, of 15 course, suitably protected by a varnishing solution, leaving it in a black and white condition, but as this adds greatly to the cost of production, it is an operation to avoid. Therefore, as already explained, I prefer to print the sound to a density 20 which will penetrate both the top and bottom emulsions. Consequently, when the film is completely colored, the sound track is composed of both red and blue. These colors, being superimposed, give the sound track an appearance of 25 more or less opaque striations on a transparent base.

In order to clearly disclose a preferred embodiment of my invention, I have hereinbefore confined the process to use with the red color image 30 on the outside of the film or in the secondary sensitized emulsion. It will be perceived that in the foregoing I have clearly disclosed a process wherein the image of the secondary emulsion or outer emulsion is first mordanted and then dyed, 35 and the underneath or primary sensitized emulsion is then toned or converted to the desired color without in any way affecting the image in the outer or secondary sensitized emulsion. Although I have hereinbefore disclosed the red 40 image on the secondary emulsion and the green-blue image on the primary emulsion, this order or placing may be reversed. The green-blue image may be imprinted in the outer or secondary emulsion, and the orange-red image may be im- 45 printed through the film 10 and in the primary or inner sensitized emulsion. In so doing, the principal steps of the process are adhered to. The outer emulsion is first mordanted and then dyed with a blue-green basic dye, after which the 50 inner or primary emulsion is converted to a red color.

The outer image may be mordanted by subjecting it to a solution having substantially the following proportions, in which potassium iodide is 55 the principal chemical:

|                  |            |
|------------------|------------|
| Iodine           | 3 grams    |
| Potassium iodide | 25 grams   |
| Acetic acid      | 4 grams    |
| Water            | 2000 c. c. |

After mordanting the outer image, it is dyed by use of a blue-green basic dye consisting essentially of a dye substance such as malachite green or one of the blue or blue-green basic dyes dissolved 60 in water to which a small amount of acetic acid has been added. The dyeing of the outer image may be accomplished in approximately five minutes, after which the film is passed through running water to clear the highlights. The inner 65 image is then red-toned by use of a uranium ton-

ing bath, which may be made up in accordance with the following formula:

|                        |            |
|------------------------|------------|
| Potassium oxalate      | 5 grams    |
| Uranium nitrate        | 5 grams    |
| Potassium ferricyanide | 5 grams    |
| Hydrochloric acid      | 2 c. c.    |
| Water                  | 1000 c. c. |

If it is necessary to print a sound record on this color positive, such sound record is printed 10 after step B, or at the time indicated at B' in the drawing, from the front or surface of the film and not through the back. In printing I do not confine the sound record necessarily to the surface emulsion but simultaneously print the primary or 15 inner emulsions in order that the final colored sound record will be represented in both red and green and will therefore approach very near to black and white.

In the foregoing description I have set forth the 20 process in what I believe to be its most practical form. I find, however, that the steps of the process may be deviated from, within reasonable limits, without seriously affecting the results to be obtained, and I contemplate that further 25 experience in the practice of the invention may develop advisable variations lying within the scope of the process hereinabove fully explained.

I claim as my invention:

1. A method of producing a color positive from 30 a film having a primary sensitized emulsion and a secondary sensitized emulsion in superposed relation, comprising: printing photographic images on said primary and secondary emulsions respectively from red and blue color value negatives; developing said images; mordanting the 35 image of said secondary emulsion for a basic dye; applying red basic dye to said secondary emulsion; removing excess of red dye from said film; blue-toning said primary emulsion by application thereto of a blue-toning solution containing ferric salts and having no affinity for the mordant carried in said secondary emulsion; and clearing said primary emulsion to render the 40 blue-toned image thereof more transparent, by 45 subjecting the film to a solution of potassium iodide.

2. A method of producing a color positive from 50 a film having a primary sensitized emulsion and a secondary sensitized emulsion in superposed relation, comprising: printing photographic images on said primary and secondary emulsions respectively from red and blue color value negatives; developing said images; mordanting the 55 image of said secondary emulsion for a basic dye by use of a solution having potassium iodide as its principal constituent; arresting the action of the mordant by subjecting it to a bisulphite solution; applying red basic dye to said secondary emulsion; removing excess of red dye from 60 said film; blue-toning said primary emulsion by application thereto of a blue-toning solution containing ferric salts and having no affinity for the mordant carried in said secondary emulsion; and clearing said primary emulsion to render the 65 blue-toned image thereof more transparent, by subjecting the film to a solution of potassium iodide.

3. A method of producing a color positive from 70 a film having a primary sensitized emulsion and a secondary sensitized emulsion in superposed relation, comprising: printing photographic images on said primary and secondary emulsions respectively from red and blue color value negatives; developing said images; mordanting the 75

image of said secondary emulsion for a basic dye by use of a solution having potassium iodide as its principal constituent; arresting the action of the mordant by subjecting it to a bisulphite solution; applying red basic dye to said secondary emulsion; blue-toning said primary emulsion by application thereto of a blue-toning solution containing ferric salts; and clearing said primary emulsion to render the blue-toned image thereof more transparent, by subjecting the film to a solution of potassium iodide.

4. A method of producing a color positive from a film consisting of a transparent base, a primary emulsion thereon, and a secondary emulsion over said primary emulsion in superposed relation, comprising: printing photographic images on said primary and secondary emulsions respectively from red and blue color value negatives; developing said images; mordanting the image of said secondary emulsion for a basic dye; applying red basic dye to said secondary emulsion; blue-toning said primary emulsion by application thereto of a blue-toning solution containing ferric salts and having no affinity for the mordant carried in said secondary emulsion; and clearing said primary emulsion to render the blue-toned image thereof more transparent by subjecting the film to a solution containing an iodide.

5. A method of producing a color positive from a film consisting of a transparent base, a primary emulsion thereon, and a secondary emulsion over said primary emulsion in superposed relation, comprising: printing photographic images on said primary and secondary emulsions respectively from red and blue color value negatives; developing said images; mordanting the image of said secondary emulsion for a basic dye by use of a solution having potassium iodide as its principal constituent; arresting the action of the mordant by subjecting it to a bisulphite solution; applying red basic dye to said secondary emulsion; removing excess of red dye from said film; blue-toning said primary emulsion by application thereto of a blue-toning solution containing ferric salts and having no affinity for the mordant carried in said secondary emulsion; and clearing said primary emulsion to render the blue-toned image thereof more transparent, by subjecting the film to a solution of potassium iodide.

6. A method of producing a color positive from a film consisting of a transparent base, a primary emulsion thereon, and a secondary emulsion over said primary emulsion in superposed relation, comprising: printing photographic images on said primary and secondary emulsions respectively from red and blue color value negatives; developing said images; mordanting the image of said secondary emulsion for a basic dye by subjecting same to a solution of substantially two grams of iodine, twenty-five grams of potassium iodide, and fifty cubic centimeters of 10% solution of acetic acid, together with sufficient water to make a total of five hundred cubic centimeters of mordanting solution; applying red basic dye to said secondary emulsion; removing excess of red dye from said film; blue-toning said primary emulsion by application thereto of a blue-toning solution having no affinity for the mordant carried in said secondary emulsion; and clearing said primary emulsion to render the blue-toned image thereof more transparent.

7. A method of producing a color positive from a film consisting of a transparent base, a pri-

mary emulsion thereon, and a secondary emulsion over said primary emulsion in superposed relation, comprising: printing photographic images on said primary and secondary emulsions respectively from red and blue color value negatives; developing said images; mordanting the image of said secondary emulsion for a basic dye by subjecting same to a solution of substantially two grams of iodine, twenty-five grams of potassium iodide, and fifty cubic centimeters of 10% solution of acetic acid, together with sufficient water to make a total of five hundred cubic centimeters of mordanting solution; applying red basic dye to said secondary emulsion, said red basic dye including substantially nine parts of chrysoidine Y, one part of safranine Y, and a small amount of acetic acid added thereto; removing excess of red dye from said film; blue-toning said primary emulsion by application thereto of a blue-toning solution having no affinity for the mordant carried in said secondary emulsion; and clearing said primary emulsion to render the blue-toned image thereof more transparent.

8. A method of producing a color positive from a film having a primary sensitized emulsion and a secondary sensitized emulsion in superposed relation, comprising: printing photographic images on said primary and secondary emulsions respectively from red and blue color value negatives; printing a single sound track through the cooperating edge portions of both of said emulsions to form identical and superimposed sound-representing images in said primary and secondary emulsions which, when subsequently toned red and blue, will produce black striations along the sound track of the positive film; developing said images; mordanting the image of said secondary emulsion for a basic dye; applying red basic dye to said secondary emulsion; removing excess of red dye from said film; blue-toning said primary emulsion by application thereto of a blue-toning solution containing ferric salts and having no affinity for the mordant carried in said secondary emulsion; and clearing said primary emulsion with a solution of soluble iodide to render the blue-toned image thereof more transparent.

9. A method of producing a color positive from a film having a primary sensitized emulsion and a secondary sensitized emulsion in superposed relation, comprising: imprinting said primary and secondary emulsions respectively with cooperating images; developing said images; mordanting the image of said secondary emulsion to receive a dye; applying a dye to said secondary emulsion; subjecting said film to a toning solution containing ferric salts to convert the image of said primary emulsion to a desired color; and clearing said primary emulsion by subjecting the film to an iodide-containing solution.

10. A method of producing a color positive from a film having a primary sensitized emulsion and a secondary sensitized emulsion, comprising: imprinting said primary and secondary emulsions respectively with cooperating images; imprinting a sound track simultaneously through both of said emulsions so that superimposed identical sound track images will be impressed on both of said emulsions; developing said images; mordanting the image of said secondary emulsion to receive a dye; applying a dye to said secondary emulsion; and then converting the image of said primary emulsion to a desired color tone.

11. A method of producing a color positive from a film having a primary sensitized emulsion and a secondary sensitized emulsion, comprising: imprinting said primary and secondary emulsions respectively with cooperating images; imprinting a sound track simultaneously through both of said emulsions so that superimposed identical sound track images will be impressed on both of said emulsions; developing said images; mordanting the image of said secondary emulsion to receive a dye; applying a dye to said secondary emulsion; and subjecting said film to a toning solution to convert the image of said primary emulsion to a desired color. 5
12. A method of producing a sound track in a color positive having primary and secondary sensitized emulsions, comprising: imprinting said primary and secondary emulsions respectively with cooperating color value images; imprinting a sound track simultaneously in both of said emulsions so that superimposed identical sound track images will be impressed on both of said emulsions; developing the images contained in said emulsions; and subsequently changing the images of said emulsions from black and white character to complementary colored images. 10
13. A method of producing a sound track in a color positive having primary and secondary sensitized emulsions, comprising: imprinting said primary and secondary emulsions respectively with cooperating color value images; from a single sound record imprinting a sound track through both of said emulsions so that superimposed and identical sound track images will be impressed simultaneously on both of said emulsions; developing the images contained in said emulsions; and subsequently changing the images of said emulsions from black and white character to complementary colored images. 15
14. A method of producing a color positive from a film having a primary sensitized emulsion and a secondary sensitized emulsion in superposed relation, comprising: imprinting said primary and secondary emulsions respectively with cooperating images; developing said images; mordanting the image of said secondary emulsion to receive a dye; applying a dye to said secondary emulsion; subjecting the film to a toning solution containing ferric salts; and clearing said primary emulsion by subjecting the film to an iodide-containing solution. 20
15. A method of producing a color positive from a film having an emulsion structure thereon of sufficient thickness to be divided into inner and outer layer portions, comprising: printing complementary photographic images on said inner and outer portions of said emulsion; developing said images; mordanting the image of said outer portion for a basic dye; applying red basic dye to said outer portion; blue-toning said inner portion of said emulsion by application thereto of a blue-toning solution containing ferric salts; and clearing said inner portion by subjecting the film to a solution of potassium iodide. 25
16. A method of producing a color positive from a film having an emulsion structure thereon of sufficient thickness to be divided into inner and outer layer portions, comprising: printing complementary photographic images on said inner and outer portions of said emulsion; developing said images; mordanting the image of said outer portion for a basic dye by use of a solution having potassium iodide as its principal constituent; arresting the action of the mordant by subjecting it to a bisulphite solution; applying red basic dye to said outer portion; blue-toning said inner portion of said emulsion by application thereto of a blue-toning solution containing ferric salts; and clearing said inner portion by subjecting the film to a solution of potassium iodide. 30
17. A method of producing a color positive from a film having an emulsion structure thereon of sufficient thickness to be divided into inner and outer layer portions, comprising: printing complementary photographic images on said inner and outer portions of said emulsion; developing said images; mordanting the image of said outer portion for a basic dye; applying basic dye to said outer portion; toning said inner portion of said emulsion by application thereto of a toning solution containing ferric salts; and clearing said inner portion by subjecting the film to a solution of potassium iodide. 35
18. A method of producing a color positive from a film having an emulsion structure thereon of sufficient thickness to be divided into inner and outer layer portions, comprising: printing complementary photographic images on said inner and outer portions of said emulsion; developing said images; mordanting the image of said outer portion for a basic dye by use of a solution having potassium iodide as its principal constituent; arresting the action of the mordant by subjecting it to a bisulphite solution; applying basic dye to said outer portion; toning said inner portion of said emulsion by application thereto of a toning solution containing ferric salts; and clearing said inner portion by subjecting the film to a solution of potassium iodide. 40
19. A method of producing a color positive from a film having an emulsion structure thereon of sufficient thickness to be divided into inner and outer layer portions, comprising: printing complementary photographic images on said inner and outer portions of said emulsion; imprinting a sound image simultaneously through both said inner and outer portions so that such sound image will be impressed in both inner and outer portions of said emulsion; developing said images; mordanting the image of said outer portion for a basic dye; applying red basic dye to said outer portion; blue-toning said inner portion of said emulsion by application thereto of a blue-toning solution containing ferric salts; and clearing said inner portion by subjecting the film to a solution of potassium iodide. 45
20. The method of producing a color photograph which includes: producing two superposed images in a photographic emulsion; developing said images; coloring the outer of said images a certain color; toning the inner of said images a substantially complementary color; and clearing said images with a solution containing potassium iodide. 50
21. The step in color toning a photograph which consists of clearing said toned photograph with a solution containing potassium iodide. 55
22. A method of producing a color positive from a film having an emulsion structure thereon of sufficient thickness to be divided into inner and outer layer portions, including: printing superimposed complementary color value images in said inner and outer portions of said emulsion; developing said images; mordanting the outer image for a basic dye; applying a blue to green basic dye to said outer image; red toning said inner image with a solution containing a uranium salt; and clearing said inner image with a solution containing potassium iodide. 60
- 75